

Feb. 20, 1923.

1,446,376

W. O. BORCHERDT

FLOTATION OF MINERALS

Original Filed June 4, 1919

3 sheets-sheet 1

Fig. 1,



INVENTOR

Walter O. Borchardt

BY

Cennie, Davis, Marvin, Edmonds

ATTORNEY

Feb. 20, 1923.

1,446,376

W. O. BORCHERDT

FLOTATION OF MINERALS

Original Filed June 4, 1919 3 sheets-sheet 2

Fig. 2



INVENTOR

Walter O. Borchardt

BY  
Pennie, Davis, Manning & Edmunds  
ATTORNEYS

Feb. 20, 1923.

1,446,376

W. O. BORCHERDT

FLOTATION OF MINERALS

Original Filed June 4, 1919 3 sheets-sheet 3

Fig. 3,



INVENTOR

Walter O. Borchardt

BY  
Rennie, Davis, Marinus & Edmonds

ATTORNEYS

## UNITED STATES PATENT OFFICE.

WALTER O. BORCHERDT, OF AUSTINVILLE, VIRGINIA, ASSIGNOR TO THE NEW JERSEY ZINC COMPANY, OF NEW YORK, N. Y., A CORPORATION OF NEW JERSEY.

## FLOTATION OF MINERALS.

Application filed June 4, 1919, Serial No. 301,832. Renewed November 27, 1922.

*To all whom it may concern:*

Be it known that I, WALTER O. BORCHERDT, a citizen of the United States, residing at Austinville, in the county of Wythe, State 5 of Virginia, have invented certain new and useful Improvements in the Flotation of Minerals; and I do hereby declare the following to be a full, clear, and exact description of the invention, such as will enable 10 others skilled in the art to which it appertains to make and use the same.

This invention relates to improvements in the differential separation of minerals by flotation, and contemplates an improved 15 method of effecting a differential separation or concentration by flotation of mixed ores, or concentrates, containing different valuable mineral constituents or species. Thus, for example, the method of the invention may be 20 advantageously employed for the production of a lead concentrate and a zinc concentrate from a mixed ore or concentrate containing lead and zinc sulfids.

I have discovered that in the presence of a 25 suitable colloid certain mineral constituents of a mixed ore pulp can be separated therefrom by flotation while the separation of other mineral constituents is inhibited. This, I believe, is due to the fact that different constituents of a mixed ore pulp differ in their adsorption capacity for colloids. 30 certain constituents having a greater absorption capacity than others due, perhaps, to their electro-positive or electro-negative 35 character, as the case may be, and to similar factors. The present invention, accordingly, involves the addition to a mixed ore pulp, substantially free of flotation-inhibitory colloidal constituents, prior to the flotation 40 treatment thereof, or to a mixed concentrate substantially free of flotation-inhibitory colloidal constituents, prior to the retreatment thereof by flotation, of a colloidal material of a suitable character and in sufficient quantity 45 to inhibit differentially the flotation of certain ingredients while permitting the flotation of others.

The invention is directly applicable to a 50 mixed ore pulp naturally so free of colloidal constituents that, if subjected to a flotation treatment in the ordinary way, a mixed concentrate of the valuable minerals would be obtained, containing these valuable minerals in approximately the same relative proportions 55 to each other as in the original ore.

Experience has demonstrated, however, that mixed ore pulps naturally so free of colloidal constituents as to show no inhibition toward the flotation of at least one of the valuable minerals therein are rare, and while 60 mixed ore pulps containing very small quantities of deleterious colloidal constituents are sometimes encountered in practice, I find it generally advantageous to subject 65 the raw or crude ore pulp to a preliminary treatment for the removal of inhibitory colloidal constituents.

Ore pulps in which there is present only 70 a single substance in colloidal condition occur less frequently than those in which, by the time the ore has been subjected to preliminary treatment such as grinding, there are 75 present two or more substances in colloidal condition. Frequently, such colloidal ingredients are released progressively as the 80 grinding or other treatment to which the ore is subjected, proceeds. In some cases these various colloidal ingredients are of opposite 85 sign or by virtue of some such property are enabled to combine with one another, forming colloidal complexes; or they mutually induce flocculation or deflocculation, or respond differently to the agents with which 90 they are treated. Thus in the lead-, zinc-, iron-, sulfid ore in dolomite gangue which occurs at Austinville, Va., there is always present 95 a certain amount of colloidal clay derived from the oxidized capping or from the oxidized zones or "water courses" occurring in the ore body. This clay colloid is already 100 free in the broken ore from the mine, and in fact, as this colloid is carried by the mine water, it is practically impossible to obtain ore which has not been brought into contact 105 with it.

The ore body also contains a certain amount of non-crystalline silica, or chert, which is perhaps a colloidal silica gel; and, in places, thin layers of an aluminous shale which appears to have been at one time a colloidal slime or mud that has become hardened or indurated by the agencies of time, heat and pressure.

While it is generally believed that a crystalline material cannot be converted into a 110 truly colloidal state by the agency of grinding only, it is well known that such materials may become colloidal if ground and weathered; and it seems obvious that a material which has once existed as a sol, and

has set but not crystallized, as for example the chert or shale above mentioned, would readily resume that state under the influence of grinding, in the presence of water containing various chemical agents.

Whatever the reason may be, I have observed that it is easier to remove the clay colloid (which I call the primary colloid) from this ore before the ore is finely ground, 10 and that the colloids derived from the fine grinding of the chert and shale (which I call the secondary colloids) yield more readily to treatment if the primary colloid has first been removed.

15 Since the clay colloid is already free in the broken mine rock, while the shale, being soft, breaks up in the preliminary operations of crushing with jaw crushers and rolls, screening, jiggling, etc., and the chert, being extremely hard and tough only breaks up, and then to a limited extent, in the final fine grinding before the flotation operation, it is relatively easy to arrange for the partial progressive separation of these colloidal constituents, and this is what is done.

It appears also that these colloidal constituents do not all inhibit the flotation of the various sulfids to the same degree, and, therefore, while differential flotation may be effected by progressively decreasing the amount of the naturally occurring colloidal constituents in an ore pulp and floating in stages, it is in some cases better to remove substantially all the colloidal constituents as 30 a preliminary operation and then effect differential flotation by adding the kind and amount of colloid to the pulp which is found by suitable laboratory testing to produce the desired inhibition of the flotation of one or more of the minerals. By so doing it is easier to secure the desired effect on the mineral the flotation of which is to be inhibited, without affecting the mineral which is to be floated and the subsequent removal of the inhibitory colloid from the tailing pulp of this flotation operation is often facilitated.

The aforementioned preliminary removal 50 of inhibitory colloidal constituents may be effected in any appropriate manner, as, for example, by deflocculating and dispersing the colloidal constituents by means of appropriate agents or other means, so that said 55 colloidal constituents assume a substantially permanent state of suspension in the water of the pulp and behave much like substances in solution, in which condition they may be removed, (with the bulk of the water of the 60 pulp) from their association with the more granular portion of the pulp by permitting the settling or sedimentation of the latter, and decanting off the colloid-bearing water; this action being facilitated, when desired, 65 by agitating the pulp in the presence of the

deflocculating agent or by heating or cooling the pulp by commonly understood means before allowing the sedimentation and decantation to take place, the latter step being conducted in tanks of the types commonly 70 used, such as the Dorr, Callow or Allen tanks, and either by overflow, displacement, or counter current decantation of the colloid-bearing water, accompanied, when desired, by dilution of the pulp with fresh water to 75 further facilitate the removal of the colloids. The preliminary removal of inhibitory colloidal constituents may also be effected by a preliminary flotation treatment under conditions permitting the removal by flotation 80 of the colloidal constituents while substantially inhibiting the flotation of the mineral particles, in which case the colloid bearing pulp is treated in a manner similar to ordinary froth flotation, but employing for the purpose of forming and stabilizing the froth an agent or agents selective for colloids rather than for metalliferous minerals, and using froth flotation apparatus of the kind 85 commonly employed, as for example the Callow cell, whereby the colloidal constituents of the pulp and a portion of the water, together with the greater part of the froth forming agent, are removed from the pulp in the form of a colloid-bearing froth, substantially free of valuable numerals, and leaving the granular residue of the pulp substantially free of colloids. In the case 90 of a mixed ore pulp containing valuable minerals, gangue and inhibitory colloids, the raw or crude pulp may be first treated for the removal of substantially all of the inhibitory colloids, for example, by either of the methods hereinbefore described, and the resulting pulp then subjected to a flotation treatment with the view of obtaining a mixed concentrate of the valuable minerals.

According to the present invention, there is added to the mixed ore pulp, or to the 100 mixed concentrate, either naturally free of inhibitory colloidal constituents or freed of such constituents as previously described, a small amount of a suitable colloid, either 105 organic or inorganic, which will differentially inhibit the flotation of certain of the mineral constituents, without inhibiting or only inhibiting to a lesser degree the flotation of certain other mineral constituents. The colloids which are added will depend 110 upon the properties of the ingredients of the ore pulp, i. e., upon the electropositive or electro-negative character of the ingredients and upon the relative attraction thereof for the added colloids, the colloidal particles 115 being commonly adsorbed by ingredients of opposite polarity. Among the colloids may be mentioned clay, in a colloidal state, or slimes such as may be obtained by decantation from ore pulps containing them; sodium 120

silicate, acacia, etc. Thus the colloidal constituents separated from the ore pulp as a preliminary operation as hereinbefore described, or some of them, may, when otherwise suitable, be recovered from the colloid-bearing water of decantation, or from the colloid-bearing froth, and after suitable purification or separation be themselves used as the colloidal agent for inhibiting the flotation of certain of the mineral constituents of the ore pulp while permitting the flotation of certain other of the mineral constituents.

In the case of the Austinville ore, one of the colloidal constituents of the ore recovered after preliminary separation as hereinbefore described has such a marked inhibitory action toward the flotation of zinc sulfid that when added to a mixed concentrate of lead and zinc sulfids obtained from this ore and the mixture subjected to froth flotation treatment in a Calow cell it permits the removal therefrom of high grade lead sulfid concentrate as the overflow froth, whilst inhibiting the flotation of the major portion of the zinc sulfid, which forms the tailings pulp of the cell, despite the fact that the mixed concentrate was itself separated from the gangue by oil flotation, and that except for the addition of the inhibitory colloid the lead and zinc sulfids seem to float with equal freedom. Colloidal precipitates may also in some cases be used, and these may be either separately formed and added to the pulp or they may be produced in the pulp by adding thereto appropriate reagents. Thus colloidal precipitates of barium sulphate, ferric oxide (or hydrate), magnesium hydrate, calcium sulphate, various silicates, etc., may be made, by means well understood, and used for the purpose of this invention.

For the selection of the best inhibitory agent in a given case simple tests based upon the principles of general and colloid chemistry are sufficient, consideration being also given to the questions of the relative amount of the various agents required, their cost and general suitability.

After the addition, and intimate incorporation of the colloid, the ore pulp is then subjected to a flotation operation, which may be carried out in apparatus of the usual types, for example, in the Calow cell, or other well known flotation machines, and with the addition of a suitable oil or other flotation agent, which will further promote the desired selective flotation of certain of its mineral constituents or ingredients.

Thereafter, the remaining ore pulp may be subjected to a treatment which will effect the dispersion or deflocculation of the colloids, if they are not already sufficiently dispersed, so that they can be removed by decantation or they may be removed by the

formation and removal of a colloid-bearing froth as hereinbefore described, and so that the ore pulp may then be again subjected to a flotation treatment for the recovery of certain other of its contained ingredients, this second flotation operation being similarly carried out with the addition of an appropriate flotation agent and in an appropriate apparatus.

For example, in the treatment of mixed lead-zinc sulfid ores where the ore pulp is naturally relatively free from colloidal matter, or has been freed of colloidal matter by the methods hereinbefore described, there may be added a small amount of a suitable colloid which will differentially inhibit the flotation of the zinc sulfid without interfering with the flotation of the lead sulfid. There may thus be added a small amount of colloidal matter, where it is of proper colloidal polarity, which has been separated from ores carrying an excess thereof, the amount of the flotation-inhibitory colloid being sufficient to bring about the desired inhibition of the flotation of the zinc. This amount can be readily determined for the particular ore by a few tests. The ore is then subjected to a flotation operation with the addition of a suitable flotation agent, for example, emulsified creosote oil, which will further promote the differential flotation of the lead sulfid.

The concentrate, as well as the tails, may be retreated in the usual manner, or the operation may be carried out in a series of flotation cells, as is common in the art. 100

After the separation of the lead concentrate, the ore pulp is then subjected to a proper treatment for the removal of a part or all of the added colloidal constituents, and is then subjected to a further concentration by flotation for the recovery of zinc sulfid. The removal of the added colloidal matter is accordingly carried out to the extent required to promote the subsequent flotation of the zinc sulfid. Where the added colloidal constituents have become flocculated or adsorbed, they may be dispersed or deflocculated by the addition of a suitable dispersing or deflocculating agent or agents which will depend in kind and amount upon the so-called colloidal polarity of the ingredients of the ore pulp and upon like considerations. I have found small amounts of sodium silicate to be well adapted to promote this dispersion with certain ores. 105

In other cases alkaline or acid agents may be indicated, or salts of various kinds, organic or inorganic, or agents which are themselves colloidal and which may be organic or inorganic. Thus I have successfully used among others, a cheap waste product of sugar manufacture known as "foun- 125

dry molasses," tri-sodium phosphate, acacia (gum arabic), sulfuric acid, caustic soda, etc.

Simple tests will serve to determine in any

- 5 specific case what agent or agents can with advantage be employed to facilitate the deflocculation or dispersion of the colloidal inhibitory agent. The major portion of the deflocculating agent will be carried out with
- 10 the decanted colloid-bearing water and the choice of agent will depend upon its effectiveness for the purpose and upon its cost, effect upon further treatment of the pulp or water and upon like considerations.
- 15 The removal of the deflocculated colloidal constituents may be effected by a simple over-flow or decantation which may be carried out on the counter-current principle, or it may be effected, with or without preliminary deflocculation of the colloids, by the formation and removal of a colloid-bearing froth, by means of suitable agents and apparatus, as previously described. For the purpose of forming a froth selective for the
- 20 colloid or colloids rather than for the metaliferous minerals, a variety of agents, organic and inorganic, are available. Simple tests will in any specific case be sufficient to determine the most suitable material, taking
- 25 into consideration the relative cost, frothing power, colloid-selective power and effect upon the subsequent treatment of the mineral pulp and the colloid-bearing froth. I have successfully used various soaps, especially those containing rosin; oils having a relatively high pitch content, and even the well-known mineral selective frothing oils, when used in excess of what would be required for mineral froth flotation, and
- 30 especially if preliminarily emulsified, are in some cases colloid-, rather than mineral-selective. Other agents, such as certain salts, or even materials which are themselves colloidal, may be used, and the greater part
- 35 of the frothing agent will in general be removed from the pulp with the froth and colloids. The ore pulp, after such further dilution as may be necessary, is then subjected to a further flotation treatment with
- 40 the aid of a suitable flotation agent or agents, for example, emulsified crude oil, pine oil and copper sulfate, and a zinc sulfid concentrate thereby obtained. The concentrate and the tailings thus produced may be
- 45 subjected to retreatment in a manner similar to that commonly practiced in the art.

In the accompanying drawings, Figs. 1, 2 and 3 are diagrammatic flow sheets illustrating, merely by way of example, three examples involving the application of the principles of the invention in the concentration of mixed ores and concentrates.

The flow sheet of Fig. 1 illustrates the application of the invention to the treatment

of a mixed ore pulp containing two different mineral constituents, designated minerals A and B on the drawing, and gangue, and substantially free of inhibitory colloids. A colloid inhibitory with respect to the flotation of mineral B is added to the pulp and is thoroughly incorporated therewith in a suitable mixing apparatus. The inhibitory colloid may be added to the ore during its preliminary treatment, as, for example, during the fine grinding, or may be added to the ore pulp that is ready for flotation. An appropriate flotation agent, preferably selective with respect to the mineral A, is introduced into the ore pulp, which is then subjected to a flotation treatment. As the result of this flotation treatment there is obtained in the over-flow froth a concentrate of mineral A, which may be retreated as desired. The tailings from the flotation treatment are then treated to remove the inhibiting colloid, as, for example, by deflocculation followed by sedimentation of the granular portion of the pulp and decantation of the inhibitory-colloid bearing water, or by the formation and removal of a colloid-bearing froth, and are then subjected to a flotation treatment in the presence of an appropriate flotation agent. The resulting concentrate of the mineral B may be retreated as desired.

The flow sheet of Fig. 2 illustrates the treatment, in accordance with the principles of the present invention, of a mixed ore pulp containing naturally sufficient colloidal material to partially or wholly inhibit the flotation of one or more valuable minerals. As indicated by the flow sheet, this ore pulp is treated, as aforementioned, for the removal of substantially all of the inhibitory colloidal matter. The resulting pulp is then subjected to a flotation treatment in the presence of an appropriate flotation agent for obtaining a mixed concentrate in which the minerals A and B are present in approximately the same relative proportions to each other as in the original ore. The minerals A and B are then separated by adding to the mixed concentrate pulp, with proper manipulation to secure intimate mixture, a colloid capable of inhibiting the flotation of mineral B and subjecting the pulp to a flotation treatment whereby the mineral A is removed in the over-flow froth, and may be retreated as desired. The tailings from this differential flotation treatment are treated for the removal of the inhibitory colloid and then subjected to a flotation treatment, in the presence of an appropriate flotation agent, thereby obtaining a concentrate of mineral B, which may be retreated as desired. Where the tailings from this last flotation treatment are in the nature of middlings, they may be returned to

the first flotation treatment, as indicated on the flow sheet.

The flow sheet of Fig. 3 illustrates the application of the invention to the treatment 5 of a mixed concentrate derived either from an ore pulp naturally free of colloids, or from one which has been sufficiently freed of colloids as hereinbefore described. A colloid capable of inhibiting the flotation of 10 mineral B is added to the mixed concentrate pulp, intimately mixed therewith, and the pulp subjected to a flotation treatment, in the presence of an appropriate flotation agent preferably selective with respect to 15 the mineral A. By this method the mineral A is removed in an overflow froth, leaving the mineral B, whose flotation has been inhibited, as the residue, which, except for its colloidal contamination, is itself a final 20 concentrate.

In ore dressing, two alternative procedures are frequently possible; (1) to treat the entire tonnage of ore by a process having a certain cost per ton, and produce, thereby, 25 tails clean enough to throw away, and concentrates good enough to keep; or (2) to treat the entire tonnage by a still cheaper process yielding tails clean enough to throw away (and generally cleaner than those produced by the first alternative), and a small 30 tonnage of low grade concentrate, which is then treated with more care by a process having a higher unit cost per ton, to yield the final concentrates. As will be readily 35 seen, the total cost for either process is the sum of the constituent products of unit cost times tonnage treated.

In the treatment of a zinc-lead-iron sulfid ore, with a dolomite gangue, such as occurs 40 at Austinville, Va., three separate colloid removals are involved. Briefly, this treatment comprises grinding all the ore, removing part of the colloid, and floating for 45 lead, and then removing more of the colloid and floating for zinc, and in addition to these two colloid removals, there is a preliminary removal to separate what I call the primary colloid, that is, the clay material 50 which is free in the ore before grinding. This involves three separate decantation operations in which the full tonnage of ore is handled each time.

In accordance with the method illustrated by the flow sheet of Fig. 2, I propose to remove, with one or two decantations, as much 55 of the colloid as is removed with the three decantations mentioned in the preceding paragraph, and to do this all before treating any of the pulp by flotation. The colloid-free 60 pulp is then treated by flotation with appropriate reagents, so as to secure the cleanest possible tails, which may be at once thrown away. The rough concentrate contains practically all of the lead and zinc, a 65 little gangue, and possibly some colloid.

This small tonnage of concentrate is then further treated, as indicated in the flow sheet of Figs. 1 or 2, depending upon how much gangue is carried over in the rough mixed concentrate, and how much colloid it 70 is necessary to add in order to secure the separation of the minerals in the mixed concentrate.

It will, accordingly, be evident that by the method represented by the flow sheet of 75 Fig. 2, the gangue is not only very cheaply eliminated, but is removed early in the concentrating process, so that in the subsequent operations only a relatively small tonnage 80 of mixed concentrates have to be dealt with. In this manner, processes can be employed for the separation of this mixed concentrate which would have so high a unit cost as to be commercially prohibitive if applied to the 85 original ore.

Throughout this specification and the appended claims, I intend to embrace, in the expressions "colloids" and "colloidal constituents," both true colloids and those quasi or borderland substances, which may not be 90 truly colloidal but partake of the qualities of, or resemble, colloids, and without regard to the sources from which such colloidal matters are derived. Thus, for the purposes of the present invention, the colloidal constituents may be considered as ranging from 95 just above the molecular size upward through the class of so-called suspensoids, which, while possibly not true colloids, still, because of their relatively large specific surface, exhibit some, if not all, of the properties of colloids, and are capable of existing in both the sol or gel state, or of being dispersed and coagulated, or flocculated and deflocculated, and exhibit flotation-inhibitory 100 effects to an extent sufficient to justify their use in the process of the present invention. 105

I claim:—

1. The method of effecting the differential flotation of minerals, which comprises adding to the mineral pulp a small amount of a colloid which of itself possesses the property of inhibiting the flotation of one mineral species of the pulp while permitting the flotation of another mineral species, and subjecting the pulp to a flotation operation. 110

2. The method of effecting the differential flotation of minerals, which comprises adding to the mineral pulp a small amount of a colloid inhibiting the flotation of certain mineral species of the pulp while permitting the flotation of another mineral species, subjecting the mineral pulp of a flotation operation, subsequently removing from the remaining pulp the added colloid to an extent 120 sufficient to promote the flotation of another mineral species of the pulp, and subjecting the pulp to a further flotation operation. 125

3. The method of effecting the differential flotation of minerals, which comprises add- 130

ing to the mineral pulp a small amount of a colloid inhibiting the flotation of certain mineral species of the pulp while permitting the flotation of another mineral species, 5 subjecting the mineral pulp to a flotation operation for the recovery of certain mineral species, adding to the remaining pulp an agent promoting the dispersion of the added colloid, separating the dispersed 10 colloid from the mineral pulp to an extent sufficient to promote flotation of other mineral species of the pulp, and subjecting the pulp to a further flotation operation for the recovery of such other mineral species. 15 4. The method of effecting the differential flotation of lead and zinc sulfids from minerals containing the same, which comprises adding to the mineral pulp a small amount of a colloid which of itself possesses the property of inhibiting the flotation of the zinc sulfid while permitting the flotation of the lead sulfid, subjecting the pulp to a flotation 20 operation for the removal of the lead sulfid, and subsequently subjecting the pulp to a further flotation operation for the removal of the zinc sulfid.

5. The method of effecting the differential separation of lead and zinc sulfids from minerals containing the same, which comprises 30 adding to the mineral pulp a small amount of a colloid inhibiting the flotation of the zinc sulfid while permitting the flotation of the lead sulfid, subjecting the pulp to a flotation operation with the aid of a flotation agent promoting the flotation of the lead sulfid, removing from the remaining pulp the added colloid to an extent sufficient to promote flotation of the zinc sulfid, and subjecting the pulp to a further flotation 35 operation with the aid of a flotation agent promoting the flotation of the zinc sulfid.

6. The method of concentrating by flotation a mixed ore pulp containing different mineral species and colloidal constituents, 45 which comprises separating the colloidal constituents from the mineral pulp, subjecting the resulting pulp to a flotation treatment and thereby obtaining a mixed concentrate of the different mineral species, 50 adding to the mixed concentrate pulp a small amount of a colloid inhibiting the flotation of certain of the mineral species of the concentrate while permitting the flotation of other mineral species, and subjecting the mineral pulp to a flotation operation. 55

7. The method of concentrating by flotation a mixed ore pulp containing different mineral species and colloidal constituents, 60 which comprises separating the colloidal constituents from the mineral pulp, subjecting the resulting pulp to a flotation treatment and thereby obtaining a mixed concentrate of the different mineral species,

adding to the mixed concentrate pulp a 65 small amount of a colloid inhibiting the flotation of certain of the mineral species of the concentrate while permitting the flotation of other mineral species, subjecting the mineral pulp to a flotation operation 70 and thereby obtaining a concentrate of the floatable mineral species, treating the tailings from the last mentioned flotation treatment for the removal therefrom of the aforementioned inhibitory colloid, and subjecting the resulting tailings pulp to a flotation operation thereby obtaining a concentrate of the floatable mineral species. 75

8. The method of concentrating by flotation a mixed ore pulp containing different mineral species and colloidal constituents, which comprises separating the colloidal constituents from the mineral pulp to an extent sufficient to promote flotation of the mineral species, subjecting the resulting pulp to a flotation treatment and thereby obtaining a mixed concentrate of the different mineral species, adding to the mixed concentrate pulp a small amount of a colloid inhibiting the flotation of certain of the 80 mineral species of the concentrate while permitting the flotation of other mineral species, subjecting the mineral pulp to a flotation operation and thereby obtaining a concentrate of a certain mineral species, treating the residue from the last mentioned flotation treatment for the removal therefrom of the aforementioned inhibitory colloid, and subjecting the colloid freed residue to a flotation treatment and thereby 85 obtaining a concentrate of another mineral species. 90

9. The method of concentrating a mixed ore pulp containing different mineral species and colloidal constituents, which 95 comprises separating the colloidal constituents from the mineral pulp, adding to the mineral pulp a small amount of a colloid inhibiting the flotation of certain mineral species while permitting the flotation of 100 other mineral species, and subjecting the mineral pulp to a flotation operation. 105

10. The method of concentrating by flotation a mixed ore pulp containing different mineral species and colloidal constituents, 115 which comprises adding to the pulp a deflocculating agent for effecting the deflocculation of the colloidal constituents, separating the deflocculated colloids from the pulp, subjecting the pulp to a flotation 120 treatment and thereby obtaining a mixed concentrate of the different mineral species, adding to the mixed concentrate pulp a small amount of a colloid inhibiting the flotation of certain mineral species thereby permitting the flotation of other mineral species, and subjecting the concentrate pulp to a flotation operation and 125

thereby obtaining a froth product containing certain mineral species and a residue containing certain other mineral species.

11. The method of concentrating by flotation a mixed ore pulp containing different mineral species and colloidal constituents, which comprises separating the colloidal constituents from the pulp, subjecting the pulp to a flotation treatment and thereby 10 obtaining a mixed concentrate of said different mineral species, adding to the concentrate pulp a small amount of a colloid inhibiting the flotation of certain of the mineral species thereof while permitting 15 the flotation of other mineral species, subjecting the concentrate pulp to a flotation operation and thereby obtaining a concentrate of one of the mineral species contained in said ore pulp, adding to the 20 residual pulp of the last mentioned flotation operation an agent promoting the dispersion of the colloids contained therein, removing the dispersed colloids from said residual pulp, and subjecting said residual 25 pulp to a flotation operation and thereby obtaining a concentrate of another mineral species contained in said ore pulp.
12. The method of concentrating by flotation a mixed ore pulp containing different 30 mineral species and colloidal constituents, which comprises separating the colloidal constituents from the pulp, subjecting the pulp to a flotation treatment and thereby obtaining a mixed concentrate of said different mineral species, adding to the concentrate pulp a small amount of a colloid inhibiting the flotation of certain mineral species thereof while permitting the flotation of other mineral species, subjecting the 35 concentrate pulp to a flotation operation and thereby obtaining a concentrate of one mineral species contained in said ore pulp, subjecting the residual pulp of the last mentioned flotation operation to appropriate 40 treatment for dispersing said added inhibitory colloid, removing the dispersed colloid from said residual pulp, and subjecting said residual pulp to a flotation operation and thereby obtaining a concentrate of another 45 mineral species contained in said ore pulp.

13. The method of effecting the differential flotation of different mineral species contained in a mixed ore pulp, which comprises adding to the pulp a small amount of 50 a colloid inhibiting the flotation of a certain mineral species thereof while permitting the flotation of another mineral species thereof, subjecting the pulp to a flotation operation for the recovery therefrom of a certain mineral species, subjecting the remaining pulp to appropriate treatment for dispersing said added inhibitory colloid and then removing the dispersed colloid from the pulp to an extent sufficient to promote 55 flotation of another mineral species of the

pulp, and subjecting the pulp to a further flotation operation for the recovery of such other mineral species of the pulp.

14. The method of concentrating by flotation a mixed ore pulp containing different 60 mineral species and colloidal constituents, which comprises separating the colloidal constituents from the pulp to an extent sufficient to promote flotation of the mineral species contained therein, subjecting the 65 thus colloid-free pulp to a flotation treatment and thereby obtaining a mixed concentrate of the different mineral species, adding to the mixed concentrate pulp a small amount of a colloid inhibiting the 70 flotation of a certain mineral species thereof while permitting the flotation of another mineral species thereof, subjecting the pulp to a flotation operation and thereby obtaining a concentrate of said certain mineral 75 species, subjecting the residual pulp from the last-mentioned flotation treatment to appropriate treatment for dispersing said added inhibitory colloid and then removing the dispersed colloid from the pulp to the 80 extent required to promote flotation of another mineral species of the pulp, and subjecting the thus colloid-free pulp to a flotation treatment and thereby obtaining a concentrate of said other mineral species. 95
15. The method of effecting the differential flotation of different mineral species in a mixed ore pulp which comprises adding to the pulp a small amount of a colloid inhibiting the flotation of a certain mineral species thereof while permitting the flotation of another mineral species thereof, subjecting the mineral pulp to a flotation operation for the recovery of said certain mineral species, subsequently removing the said 100 added inhibitory colloid in a dispersed condition from the remaining pulp to the extent required to promote the flotation of another mineral species of the pulp, and subjecting the pulp to a further flotation 105 operation for the recovery of said other mineral species thereof. 110

16. The method of concentrating by flotation a mixed ore pulp containing different mineral species, which comprises subjecting the ore pulp to a flotation treatment and thereby obtaining a mixed concentrate of the different mineral species, adding to the mixed concentrate pulp a small amount of a colloid which of itself possesses the 115 property of inhibiting the flotation of certain mineral species thereof, while permitting the flotation of other mineral species, and subjecting the mineral pulp to a flotation operation and thereby obtaining a froth 120 product containing certain mineral species and a residue containing certain other mineral species.

In testimony whereof I affix my signature.  
WALTER O. BORCHERDT,